

## UNITED STATES PATENT OFFICE

2,132,929

## SPINNING SOLUTION

Rudolph S. Bley, Elizabethton, Tenn., assignor to  
North American Rayon Corporation, New York,  
N. Y., a corporation of Delaware

No Drawing. Application December 2, 1937,  
Serial No. 177,824

12 Claims. (CL 106—40)

In the manufacture of cellulosic products, such as filaments, threads, and the like, a viscose solution is continuously extruded through the minute orifices of a spinneret into a coagulating or setting bath. However, since the introduction of the viscose process great troubles have been and are still experienced as far as continuous spinning is concerned due to impurities, such as, for example, precipitated cellulose particles, sulphur and resin particles, zinc compounds, etc., present in either the viscose solution or the spin bath. These impurities gradually contaminate the spinnerets, clog and reduce the widths of the spinneret holes with the result that filaments of uneven thickness are obtained. If contamination of the spinnerets and clogging of their holes proceeds the individual filament start to tear and occasion interruption of the spinning process.

By experimentation, I have found that contamination of spinnerets and clogging of spinneret holes may be overcome by spinning viscose solutions in the presence of cation-active compounds, these compounds being produced by condensing a halogenated petroleum hydrocarbon, having a chain of eight or more carbon atoms, with a tertiary base selected from the group consisting of amines, phosphines, arsines and stibines, or with an organic sulphide selected from the group consisting of dialkyl sulphides, diaryl sulphides, and alkyl-aryl sulphides under substantially anhydrous conditions.

Petroleum consists of complex mixtures of hydrocarbons concerning the chemical nature of which there is very little information, although there are indications that all of these materials contain members of the methane series, the polymethylene series and the benzene series of hydrocarbons. The difference between petroleum of various sources resides in the proportions of the different types of hydrocarbons and in the chemical nature and amounts of their impurities. Pennsylvania oil, for example, contains a large proportion of methane hydrocarbons and practically no impurities of sulphur or nitrogen compounds. About thirty hydrocarbons have been isolated and identified with certainty. Distillation is the principal method used in separating crude petroleum into useful components. The distilled fractions from crude petroleum are casinghead gasoline, gasoline, kerosene, gas oil and lighter lubricating oils (" neutrals"). The residues from such distillation supply most of the lubricating oils ("bright stock"), petrolatum in pasty or liquid form and either paraffin wax or petroleum pitch, depending upon the nature

of the crude petroleum. Kerosene is any mixture of hydrocarbons which is not volatile enough for use as gasoline in explosion motors. Cracked gasolines are rich in olefins and diolefins. Paraffin wax was originally obtained from tars from the distillation of wood, peat, and lignite, but is now obtained from petroleum, and especially from Pennsylvania paraffin-base oils. Little information is available about the composition of paraffin waxes except that it consists mainly of higher alkanes and only small amounts of the normal compounds. Petrolatum (Vaseline) is a pasty mixture of hydrocarbons similar to paraffin while liquid petrolatum is a high boiling petroleum distillate. Ozokerite is a natural paraffin wax originating in Galicia; in bleached form it is termed "ceresin". All of these petroleum hydrocarbons may be halogenated in conventional manner in the presence or absence of catalysts to form halogenated hydrocarbon mixtures adapted to be condensed with the tertiary bases and organic sulphides, set forth above. The hydrocarbonaceous materials i. e., crude petroleums, casinghead gasolines, gasolines, kerosenes, gas oil, lubricating oils, pasty and liquid petrolatums and paraffin waxes, to be halogenated may first be dissolved in carbon tetrachloride, etc., and subsequently chlorine, bromine, etc., in gaseous form introduced therein until the heat of reaction abates. Halogenated compounds, containing about 25 to 40% of halogen may be obtained in this manner. However, upon prolonging the introduction of halogens, compounds may be obtained containing up to about 75% of a halogen, and it is to be noted that the boiling or fusing points of the raw materials are either lowered or raised by halogenation. Hydrochloric acid, hydrobromic acid, etc., formed during this reaction must be removed, preferably by neutralization. Catalysts, such as iron, etc., may be added to the mixtures to accelerate halogenation. Halogenation will also proceed more rapidly by carrying out the reaction under the influence of ultra-violet rays. The halogenation may also be performed in accordance with processes disclosed, for example, in U. S. Patent #989,225 to Blakeman of April 11, 1911; U. S. Patent #1,191,916 to Brooks of July 18, 1916; U. S. Patent #1,246,810 to Ellis of November 13, 1917; U. S. Patent #1,432,761 to Koch of October 24, 1922; etc. Chlorinated paraffin wax, sold under the trade name of "Chlorafin" is a very suitable raw material for my process.

Tertiary bases, capable of being condensed with the halogenated hydrocarbonaceous materials,

set forth above, are for example: Trialkyl amines, dialkyl-aryl amines, alkyl-diaryl amines, triaryl amines, pyridine, substituted pyridines, pyridazine, pyrimidine, pyrazine, triazole, oxazole, 5 tetrazole, quinoline, substituted quinolines, acridine, substituted acridines, phenanthridines, phenanthrolines, phenazine, picoline, substituted picolines, trialkyl phosphines, dialkyl-aryl phosphines, alkyl-diaryl phosphines, triaryl phosphines, trialkyl arsines, dialkyl-aryl arsines, alkyl-diaryl arsines, triaryl arsines, trialkyl stibines, dialkyl-aryl stibines, triaryl stibines, etc. Organic sulphides suitable for being condensed with these halogenated petroleum hydrocarbons 10 are dialkyl sulphides, alkyl-aryl sulphides and diaryl sulphides. Thus, during such condensations cation-active ammonium, phosphonium, arsonium, stibonium and sulphonium compounds are obtained which are capable of preventing the 15 incrustation of spinnerets and spinneret holes through which viscose solutions are extruded into a spin bath. Cation-active compounds are surface-active compounds which carry in the cation a hydrocarbon chain having eight or more carbon atoms. They are particularly advantageous 20 because they may be used in neutral salt, alkaline and acidic aqueous solutions and also in hard water. In contradistinction to cation-active compounds, anion-active compounds are surface- 25 active compounds which carry in the anion a more or less extended hydrocarbon chain. They flocculate in neutral salt, alkaline and acidic aqueous solutions, and also in hard water. Common soaps, sulphonated oils, etc., are anion-active compounds, and thus they are unable to prevent the 30 incrustation of spinnerets and spinneret holes. These incrustation inhibitors are prepared by 35 heating a halogenated hydrocarbonaceous material of the group, set forth above, with a tertiary amine or an organic sulphide at a moderate temperature—preferable under reflux—until condensation is completed. Before heating the two components they may be dissolved in a suitable, inert solvent, such as, for example, benzene, 40 ether, toluene, etc., i. e., in solvents which are incapable of chemically reacting with the compounds to be condensed. The inert solvent may subsequently be removed from the condensation products by distillation and the unreacted base 45 or sulphide separated from the condensation products by distillation, extraction, etc. The crude incrustation inhibitors may contain a number of different condensation products which need not be separated from each other. In other 50 words, the crude condensation products (incrustation inhibitors) containing surface-active and surface-inactive constituents may be added for reasons of economy without further purification to viscose solutions or spin baths (setting baths). 55 Although these cation-active halides, i. e., bromides, chlorides, fluorides and iodides, may form corresponding bases in viscose solutions and salts in spin baths, they retain their surface-activity and, thus, their property of preventing incrustations. If very small amounts of these 60 condensation products are added to viscose solutions or spin baths the physical characteristics, such as strength, plasticity, lustre, etc., of regenerated cellulose produced therefrom or there- 65 in remain unaltered. Upon increasing the amount of incrustation inhibitor in a given viscose solution or spin bath, the regenerated cellulose produced therefrom or therein, respectively, 70 may alter its physical characteristics, i. e., it 75 may acquire a soft-lustre, become more plastic,

lose part of its original strength, etc. For such reasons, the amounts to be added to viscose solutions or spin baths must be pre-determined by experimentation. Additions of about 0.4 to 1 gram per liter of viscose solution or spin bath are sufficient to allow continuous spinning without substantially changing the inherent physical characteristics of regenerated cellulose.

Although these cation-active petroleum derivatives improve the spinning properties of any conventional viscose solution or spin bath, I have found that they are especially valuable as additions to zinc-bearing spin baths, i. e., spin baths containing a zinc compound, such as, for example, zinc sulphate, these baths having poor spinning 1 qualities.

#### Example I

About 10 grams of a halogenated petroleum are mixed with about 50 grams of triethanolamine and heated under reflux at a moderate temperature, i. e., a temperature at which the raw materials as well as condensation products formed therefrom remain stable, until condensation is complete. About 0.4 to 1 gram of the reddish-brown condensation product are added to one liter of a viscose solution of conventional concentration and maturity. This solution is then extruded into an acid spin bath, such as, for example, a glucose bath, a magnesium-zinc bath, etc. The spinnerets and spinneret holes remain clean on prolonged spinning. Other ammonium as well as phosphonium, arsonium, stibonium and sulphonium compounds, prepared as set forth above, may be used with equal success.

#### Example II

A conventional viscose solution is extruded through fine orifices in precious metal spinnerets into an acid spin bath, containing sulphuric acid, sodium sulphate, ammonium sulphate and zinc sulphate and about 0.5% by weight of a cation-active substance prepared by heating (condensing) a chlorinated paraffin or other halogenated hydrocarbonaceous material with pyridine. Spinning irregularities and difficulties are substantially overcome. Without the addition of these incrustation inhibitors, spinning is interrupted after a very short period of time.

#### Example III

The cation-active compound is added to both the viscose solution and the spin bath following Examples I and II.

Although these examples will serve to illustrate the present invention, I do not wish to be limited to the inhibitors and concentrations thereof recited therein, since I may make use of any cation-active ammonium, phosphonium, arsonium, stibonium or sulphonium compound prepared by condensing a halogenated material containing at least one petroleum hydrocarbon having eight or more carbon atoms in its chain selected from the group consisting of crude petroleums, gasolines, kerosenes, lubricating oils, pasty and liquid petrolatums and paraffin waxes with a tertiary amine selected from the group consisting of amines, phosphines, arsines and stibines or an organic sulphide selected from the group consisting of dialkyl sulphides, diaryl sulphides and alkyl-aryl sulphides under substantially anhydrous conditions, provided these cation-active compounds are sufficiently soluble in either viscose solutions or spin baths to furnish cations therein.

Modifications of my invention will readily be

recognized by those skilled in the art, and I desire to include all such modifications coming within the scope of the appended claims.

I claim:

5. 1. A spinning solution for the production of artificial products comprising a viscose solution and a cation-active condensation product of a halogenated hydrocarbonaceous material selected from the group consisting of halogenated crude 5 petroleums, halogenated gasolines, halogenated kerosenes, halogenated lubricating oils, halogenated pasty petrolatums, halogenated liquid petrolatums and halogenated paraffin waxes and a tertiary base selected from the group consisting 10 of tertiary amines, tertiary phosphines, tertiary arsines and tertiary stibines, said condensation product being sufficiently soluble in said viscose solution to become cation-active therein.
15. 2. A spinning solution for the production of artificial products comprising a viscose solution and a cation-active condensation product of a halogenated paraffin wax and triethanolamine.
20. 3. A spinning solution for the production of artificial products comprising one liter of a viscose solution and about 0.4 to 1.0 gram of a cation-active condensation product of a halogenated hydrocarbonaceous material selected from the group consisting of halogenated crude 25 petroleums, halogenated gasolines, halogenated kerosenes, halogenated lubricating oils, halogenated pasty petrolatums, halogenated liquid petrolatums and halogenated paraffin waxes and a tertiary base selected from the group consisting of tertiary amines, tertiary phosphines, tertiary arsines and tertiary stibines, said condensation product being sufficiently soluble in said viscose solution to become cation-active 30 therein.
35. 4. A spinning solution for the production of artificial products comprising one liter of a viscose solution and about 0.4 to 1.0 gram of a cation-active condensation product of a halogenated paraffin wax and triethanolamine.
40. 5. A soft-lustre regenerated cellulose containing a finely divided cation-active condensation product of a halogenated hydrocarbonaceous material selected from the group consisting of halogenated crude 35 petroleums, halogenated gasolines, halogenated kerosenes, halogenated lubricating oils, halogenated pasty petrolatums, halogenated liquid petrolatums and halogenated paraffin waxes and a tertiary base selected from the group consisting of tertiary amines, tertiary phosphines, tertiary arsines and tertiary stibines, said condensation product being sufficiently soluble in said viscose solution to become cation-active 40 therein.
45. 6. A soft-lustre regenerated cellulose containing a finely divided cation-active condensation product of a halogenated paraffin wax and triethanolamine in a sufficient amount to diminish 45 the lustre thereof.
7. A spinning solution for the production of artificial products comprising a viscose solution and a cation-active condensation product of a 15 chlorinated paraffin wax and triethanolamine.
8. A spinning solution for the production of artificial products comprising a viscose solution and a cation-active condensation product of a chlorinated paraffin wax and a tertiary amine, said 20 condensation product being sufficiently soluble in said viscose solution to become cation-active therein.
9. A spinning solution for the production of artificial products comprising one liter of a viscose solution and about 0.4 to 1.0 gram of a cation-active condensation product of a chlorinated paraffin wax and triethanolamine.
10. A spinning solution for the production of artificial products comprising one liter of a viscose solution and about 0.4 to 1.0 gram of a cation-active condensation product of a chlorinated paraffin wax and a tertiary amine, said 25 condensation product being sufficiently soluble in said viscose solution to become cation-active 30 therein.
11. A soft-lustre regenerated cellulose containing a finely divided cation-active condensation product of a chlorinated paraffin wax and triethanolamine in a sufficient amount to diminish 40 the lustre thereof.
12. A soft-lustre regenerated cellulose containing a finely divided cation-active condensation product of a chlorinated paraffin wax and a tertiary amine in a sufficient amount to diminish 45 the lustre thereof.

RUDOLPH S. BLEY.